# EUROPEAN PATENT SPECIFICATION

(11) **EP 0 151 836 B1**
(45) Date of publication and mention of the grant of the patent: **11.05.1988**
(21) Application number: 84300719.6
(22) Date of filing: 06.02.1984
(51) Int. Cl.: B65H 55/00

(54) **Yarn package of carbon filament yarn and method for forming the same**
Kohlenstoffilament-Garnwickel und Verfahren zum Herstellen desselben
Enroulement de fil de filament en carbone et procédé pour l'obtention d'un tel enroulement

(43) Date of publication of application: 21.08.1985
(73) Proprietor: TORAY INDUSTRIES, INC., Tokyo 103 (JP)
(72) Inventor: Yamamoto, Ryuichi, Iyo-gun Ehime-ken (JP); Nojiri, Hironobu, Iyo-gun Ehime-ken (JP)
(74) Representative: Ellis, John Clifford H.

(56) References cited:
- CH-A- 318 773
- DE-A- 2 027 005
- FR-A- 770 433
- GB-A- 935 299
- US-A- 2 639 872
- US-A- 3 666 200

## Description

### Background of the invention

This invention relates to an improved package of carbon filament yarn, which can be smoothly unwound without generation of fluff and yarn breakage.

As is well known to the person skilled in the art, carbon filament is nowadays utilized as a basic component for combination with resins or metals to form a reinforced composite matrix. Most carbon filament is produced by heat-treating multi-filaments of acrylonitrile synthetic fiber or so-called "pitch fiber" in an oxidizing atmosphere at a temperature of 200°C to 400°C for imparting an anti-flame property, and then heating them in an inert atmosphere at a temperature of 800°C to 2800°C for carbonization. As with conventional synthetic fiber, the resultant carbon filament is often wound on a bobbin to form a yarn package of a square-end cheese type for easy handling.

In FR-A-770433, which dates from 1934, a period before the introduction of carbon filaments, it was explained that regular or patterned windings were almost always avoided in the production of cross-wound bobbins. The invention of that patent was the production of cross-wound bobbins having a regular or patterned winding, in which the thread was displaced by of a complete revolution of the bobbin at each displacement stroke of the thread on the periphery of the bobbin, where

In the above equation p, q, r and s are integers, are irreducible fractions, p is less than q, r is at least 300 times smaller than s, q is less than 30 and s is larger than 500.

A carbon filament, however, has properties quite different from conventional synthetic textile filaments, that is, the carbon filament has an extremely high Young's modulus, very low elongation, and weakness for bending as well as an extremely high surface smoothness compared to those of the textile filaments. This means that a carbon filament yarn has a less ability of self-adjusting in a winding operation. Therefore, it is difficult to control winding conditions for forming a package of carbon filament yarn with a winder, particularly, a winding tension of the yarn to obtain a good package of carbon filament yarn. For example, when a carbon filament yarn package is formed under a low winding tension, the yarn tends to slip over from the shoulders of the package. On the other hand, a high winding tension causes breakage of component filaments of the yarn during the winding operation, resulting in considerable fluff in the package.

Further, increased consumption of carbon filament has led to demands for large packaging, such as packages of 1 to 10 kg in weight. The larger the package, however, the greater the above-mentioned drawbacks. Even if a properly shaped package can be obtained, the yarn tends to slip over from the shoulders upon transport or in an unwinding process, because the package is very sensitive to mechanical shock and the yarn portions distributed therein easily move in relation to each other. With a deformed package, breakage of component filaments of the yarn and fluff may occur during the unwinding operation.

In another area, the heat-treating process is a bottleneck in the production of carbon filament, because the process has to be carried out at a low temperature of 200°C to 400°C for a long period, such as from several ten minutes to several hours. If the process is carried out at a higher temperature to reduce the processing time, serious trouble such as combustion or explosion may occur due to a run-away reaction. Under such circumstances, it is convenient to treat a plurality of carbon filament yarns in parallel in the furnace to increase productivity.

When treating a plurality of carbon filament yarns in parallel, a so-called "multi-cop winder" having a long spindle supported in a cantilever manner and a pressure roll provided along the spindle, on which spindle a plurality of bobbins are held longitudinally, may be utilized to take up the resultant carbon filament yarns. In the multi-cop winder, however, it is difficult to control the winding conditions of the packages on the spindle, whereby a difference in quality may arise between the resultant packages, In the case of large packaging, the spindle tends to bend due to the increased weight of the packages thereon, and the pressure acting between the surface of the packages and the pressure roll. Naturally, the displacement according to the bending is maximum at the free end portion of the spindle and decreases toward the root portion thereof. This causes a difference between the packages in the running yarn length between the fulcrum of yarn traversing and the surface of the package, and this causes a large difference in winding tension between the packages. In case of winding of the conventional textile yarn, the difference between the packages in the running yarn length between the fulcrum of yarn traversing and the surface of the package does not substantially cause a difference in winding tension between the packages; however, in case of winding of the carbon yarn, it causes a large difference in winding tension between the packages, since the carbon yarn has very high Young's modulus compared to that of the textile yarn. The difference in winding tension tends to produce a package wound under an undesirable high winding tension or an undesirable low winding tension.

### Summary of the invention

It is an object of the present invention to provide a yarn package of carbon filament of good shape, which, in spite of large packaging, does not substantially deform during transport or unwinding and ensures less breakage of component filaments of the yarn and less fluff.

It is another object of the present invention to provide a method for forming the above package.

The above-mentioned objects of the present invention are achievable by a square-end cheese type yarn package of carbon filament yarn comprising a bobbin and a continuous carbon filament yarn wound on the bobbin with a plurality of yarn traces imparted by a repeated traverse motion. The yarn trace imparted by the traverse motion is repeated every n cycles at a shifting ratio within a range of from 50% to 150% relative to an average yarn width, where n is a positive integer selected from a range of from 1 to 9.

The yarn package according to the present invention preferably has the shifting ratio within a range of from 75% to 125% and/or the cycles being within a range of from 2 to 6. The yarn package according to the present invention preferably has an initial winding angle of not more than 30°, more preferably not less than 10° and further more preferably not more than 17°, and a final winding angle of not less than 4°, more preferably not more than 12° and further preferably not less than 5°. The yarn package according to the present invention preferably has an average yarn width within a range of from 1 mm to 5 mm, more preferably within a range of from 2 mm to 4 mm. The yarn package according to the present invention preferably has a wound yarn volume of more than 0.04 kg per cm (0.1 kg per inch) of the package width and package hardness within a range of from 50° to 85°, more preferably within a range of from 65° to 75°.

The above package can be obtained by utilizing a spindle drive winder comprising a positively rotatable spindle supported in cantilever fashion, a bobbin fitted on the spindle, a freely rotatable pressure roll provided along the spindle and a yarn traversing guide for reciprocating the yarn in the direction of the axis of the bobbin, whereby a carbon filament yarn is wound on the bobbin or bobbins fitted on the spindle with a constant winding ratio to form the package or packages, characterised in that the winding ratio (as hereafter defined) is selected so that a yarn trace on the package formed by a traverse is repeated every n cycles at a shifting ratio within a range of from 50% to 150% relative to an average yarn width, n being a positive integer selected from a range of from 1 to 9.

In the above method, the winding tension is preferably within a range of from 0.03 g/D to 0.3 g/D, more preferably from 0.07 g/D to 0.2 g/D at the initial stage of the winding operation and preferably within a range of from 0.015 g/D to 0.3 g/D, more preferably from 0.03 g/D to 0.2 g/D at the final stage of the winding operation.

A multi-cop winder comprising a spindle having an effective length more than 400 mm is favourably utilized for carrying out the inventive method. In this case, the package having a weight of more than 0.04 kg per cm (0.1 kg per inch) of package width is formed under the condition that a deviation of the spindle relative to a pressure roll is within a range of from 1/5000 to 1/500.

In this case, further, a gap between a pressure roll and a surface of each package on the spindle is kept preferably within 2.0 mm, the variance thereof being within 0.2 mm.

### Brief description of the drawings

The present invention will be apparent from the description of embodiments according to the invention with reference to the accompanying drawings, in which
Fig. 1 is a perspective view of a conventional spindle drive type winder utilized for carrying out the present invention;
Fig. 2A is an enlarged view of a mesh-like crossing pattern appearing on the surface of a yarn package when a yarn shifting ratio is 50% of the yarn width;
Fig. 2B is a similar view as Fig. 2 when a yarn shifting ratio is 150% of the yarn width;
Fig. 3 is a schematic plan view of a multi-cop winder utilized for carrying out the present invention; and
Fig. 4 is a diagram of the clearance between a spindle and a pressure roll of the multi-cop winder shown in Fig. 3 for explaining a deviation therebetween.

### Description of the preferred embodiment

A yarn package 1 of carbon filament yarn is formed by means of a conventional spindle drive winder shown in Fig. 1. The winder comprises a spindle 3, one end of which is rotatably supported in a housing 2 accommodating a means for driving the spindle, such as a torque motor (not shown), and the other end being free, and a pressure roll 4 disposed parallel to the spindle 3 in a freely rotatable manner.

In the vicinity of an outer surface of the pressure roll 4 is a traverse guide 5 engaged with a scroll groove of a traverse cam (not shown) so as to be able to move reciprocatively on a predetermined path arranged parallel to the spindle 3. A carbon filament yarn Y which is preferably originated from acrylonitrile synthetic fiber is delivered from a preceding process, such as a carbonization, at a constant rate and is taken up, through the traverse guide 5 on a bobbin 6 fitted on the spindle 3, whereby a cross-wound package 1 of a square-end cheese type is obtained. As the diameter of the package 1 increases, a rotational speed of the spindle 3 is controlled to decrease so that a peripheral speed of the package 1 can be kept constant. The spindle 3 also displaces away from the pressure roll 4 by being guided by means of a dog-segment 8 provided on a wall of the housing 2, to which a dog 7 of the spindle 3 is slidably engaged, so that a gap between the surface of the package 1 and the pressure roll 4 can be kept constant (the gap is preferably less than 1 mm). A function of the pressure roll 4 is to gradually level unevenness on the package surface and to control the hardness of the package.

Basically, the yarn is distributed on the package surface in a ribbon shape by the traverse motion, forming a yarn trace on the package surface each traverse. The successive yarn traces cross with each other to form a mesh-like crossing pattern 10 on the package surface as shown in Figs. 2A and 2B. The yarn portions in the package can be retained in their given positions by this intercrossing.

The present inventors have found that the desired yarn package can be obtained by controlling the position of the yarn trace. That is, the desired package can be obtained by ensuring that each yarn trace is formed close to a prior trace formed a few number of traverses before. The yarn traces are not desirably formed at exactly corresponding positions since the resultant overlapping of yarn portions would result in an uneven package surface. Therefore, it is necessary to shift the yarn traces from each other with a shifting ratio of from 50% to 150%, preferably from 75% to 125%, relative to the yarn width. The corresponding yarn traces must be formed within not more than nine, preferably in a range of from 2 to 6, traverses. The yarn width is preferably in a range of from 1 mm to 5 mm in average, more preferably in a range of from 2 mm to 4 mm.

If the shifting ratio is less than 50%, namely, if a yarn trace is wound onto the corresponding prior trace with an overlapped distance more than a half of the yarn width, the filaments in the yarn tend to entangle upon unwinding from the resultant package, which causes considerable fluff in the yarn. Further, the surface of the package becomes uneven due to so-called "ribbon wind", which results in a deformed package having a low apparent density.

On the other hand, if the shifting ratio exceeds 150%, namely, if the two yarn traces have a gap 11 (see Fig. 2B) wider than a half of the yarn width, the yarn portion tends to slip on the package due to lack of constraint force, also causing a deformed package. This phenomenon becomes more evident in forming larger packages.

The shifting ratio is preferably selected to in accordance with the yarn thickness. For example, the shifting ratio is preferably from 50% to 100% relative to the yarn width for yarn of about 3600 total denier and from 100% to 150% for yarn of about 7200 total denier. Generally speaking, a larger shifting ratio is preferable for larger yarn width.

Figures 2A and 2B show mesh-like crossing patterns corresponding to shifting ratios of 50% and 150%, respectively.

A method for forming the package is described below. The package is formed by using the spindle drive winder illustrated in Fig. 1. This winder is of a constant winding ratio type, that is, a predetermined winding ratio is maintained throughout the winding operation, while the winding angle gradually decreases as the diameter of the package increases. Here, the winding ratio means the number of revolutions of the package during one cycle of yarn traverse along the bobbin.

The desired shifting ratio is obtained by selecting a suitable winding ratio. A method forthe selection is explained below:

A winding ratio Wₒ, calculated without consideration of yarn width is determined by equation (1) where L is traverse width in mm, Do is an outer diameter of a bobbin in mm, and 8 is an initial winding angle.

An adjusting value dW is determined by equation (2) where y is a shifting distance in mm and n is the integer mentioned before.

The desired winding ratio W, is calculated by equation (3)

In equation (3), W, obtained from (Wₒ-dW) is preferably used.

In the above case, the initial winding angle is preferably selected to be in a range of from 10° to 30°, which corresponds to a final winding angle of from 4° to 12°. This is because, if the winding angle exceeds the above range, a bulge tends to develop on the shoulders of the package, which damages the yarn. On the other hand, if the winding angle is below the range, the yarn on the package tends to slip over from the shoulders.

A suitable winding ratio W₁, when a yarn of 2 mm width is wound on a bobbin of 82 mm diameter with a traverse width of 152 mm, a winding angle of 15° and a shifting ratio of 75% is calculated by equations (1), (2), and (3) as follows:

When the winding operation is carried out under a winding ratio of 4.3957 adjusted according to the invention, the yarn package is formed in such a manner that the yarn trace is repeated with a shifting ratio of 75% relative to the average yarn width. Actually, the winding ratio is selected, with reference to the above calculated result, from the group of suitable gear combinations listed on the table attached to the winder.

### Example 1

Two carbon filament yarns with yarn widths of 2.0 mm and 4.0 mm, respectively, were wound to form packages under various shifting ratios. The resultant packages were examined for their appearance and unwinding smoothness. The results are shown in Table 1.

As apparent from Table 1, packages No. 1, 2, and 4, formed with shifting ratios according to the present invention, showed good appearance and excellent unwinding smoothness.

The package according to the present invention preferably has a hardness in a range of from 50° to 85°, more preferably from 65° to 75°, especially when it is formed of a yarn having a total denier (D) within a range of from 500 to 20000 and is of a weight of more than 0.04 kg per cm (0.1 kg per inch) of the package width. The hardness referred to herein is a value measured a Model C Hardness Tester provided by Kobunshi Keiki Seisakusho, Japan. Three circumferentially spaced points on each of the two shoulders and a center of the package surface were selected as measured points. The average value was utilized as a representative of the package hardness.

If the hardness is smaller than 50°, the package is poor in appearance and tends to be deformed by slipping-over. On the other hand, if the hardness exceeds 85°, the yarn portion in the package tends to adhere to the adjacent portion, whereby smooth unwinding thereof cannot be expected. Thus, a hardness of from 50° to 85° assures a good appearance and smooth unwinding of the package as well as possibility of large packaging.

In order to obtain a package with a hardness within a range of from 50° to 85°, the winding tension of the yarn has to be controlled to within a range of from 0.03 g/D to 0.3 g/D at the first stage of the winding operation and to within a range of from 0.015 g/D to 0.3 g/D at the final stage thereof. Further, to obtain a package with a hardness in a range of from 65° to 75°, the winding tension has to be controlled to within a range of from 0.07 g/D to 0.2 g/D at the first stage and to within a range of from 0.03 g/D to 0.2 g/D at the final stage. The winding tension may be constant throughout the winding operation, but preferably decreases in accordance with the progress of the winding operation as described above.

### Example 2

A carbon filament yarn having a total denier of 3000 composed of 6000 filaments was wound by the winder shown in Fig. 1 with six initial tensions in a range of from 0.01 g/D to 0.4 g/D and with final tensions controlled to be a half of the initial tensions. Packages were obtained corresponding to the six tension modes.

The properties of the packages were tested. The results are indicated in Table 2.

As apparent from the table, in the case of a lower initial tension of 0.01 g/D, the yarn on the growing package tended to slip-over. Therefore, a volume of wound yarn of more than 0.012 kg-weight per cm (0.3 kg per inch) of the package width could not be obtained. Contrary to this, the package wound with an initial tension of 0.4 g/D had a hardness of more than 90°, which generated considerable fluff during the unwinding thereof. Thus, the initial winding tension is preferably within a range of from 0.03 g/D to 0.3 g/D, more preferably, from 0.07 g/D to 0.2 g/D.

Another aspect of the present invention carried out by means of a multi-cop winder illustrated in Fig. 3 will now be explained.

The multi-cop winder is substantially of the same construction as the spindle winder shown in Fig. 1, except that the former has a longer spindle 3 supported in a cantilever manner. A plurality of bobbins (in this case, four bobbins) are mounted thereon corresponding to each yarn to be wound to form packages 1 a to 1d. The multi-cop winder is preferably utilized for simultaneously winding a plurality of carbon filament yarns delivered from the carbonizing furnace at a relatively slow speed, so that the overall productivity of the process is increased.

A function of the pressure roll 4 is to level unevenness of the surface of a package, as stated before. In the multi-cop winder, another very important function is to impart a constant surface pressure (preferably within a range of from 0.1 to 0.3 kg/cm) onto all the packages on the spindle to obtain uniform size packages. For this purpose, the gap between the package surface and the pressure roll has to be kept less than 2.0 mm, preferably less than 1 mm, and the variance thereof has to be kept within 0.2 mm, otherwise the hardness of the resultant package may fluctuate more than 5%. However, in case of a longer spindle, the effective length of which exceeds 400 mm, the spindle 3 tends to bend due to the counter force acting on the packages from the pressure roll 4 as well as the increasing weight of the packages. Here, the effective length means a length from a free end of the spindle to a root portion thereof emerging from a bearing supporting the spindle. Therefore, the free end portion of the spindle gradually bends away from the pressure roll, causing a difference in surface pressures between the packages. This causes a difference of diameters between the packages on the spindle. Since the carbon filament yarn has a high Young's modulus, such a diameter difference results in the great difference of the winding tensions for the package, especially in the final stage of the winding operation. It is apparent that the thus obtained packages may include low quality ones, as stated before.

To prevent this, according to the present invention, the relative positions of the spindle and the pressure roll are previously deviated to be nonparallel, so as to compensate for the bending of the spindle especially at the final stage. The deviation may be provided so that the gap between the root portions of the spindle and of the pressure roll is greater than that between the free end portion of the spindle and the pressure roll. It is also possible to adjust the spindle so that the free end thereof is positioned above the normal level relative to the pressure roll with or without the above deviation of the root portion of the spindle.

The dimensional relationship of the spindle and the pressure roll is explained in detail referring to Fig. 4. The deviation A of the spindle 3 from an imaginary line parallel to the pressure roll 4 is defined by the following equation where I is an effective length of the spindle 3, and W and W' are gaps between the spindle 3 and the pressure roll 4 at the free end portion and the root portion thereof, respectively. The deviation A is preferably within a range of from 1/5000 to 1/500. Of course, the direction of this deviation is decided by taking that of the resultant force which causes the bending of the spindle into account, so that the deviation can cancel the bending throughout the winding operation.

### Example 3

Four carbon filament yarns each having a total denier of 3000 and composed of 6000 filaments were simultaneously taken up by the multi-cop winder shown in Fig. 3 without prior adjustment of the spindle under an initial winding tension of 0.2 g/D and a final winding tension of 0.1 g/D. The winding operation was carried out until the volume of wound yarn reached a weight of 0.4 kg per cm (1.0 kg per inch) of package width. The winder was controlled to maintain the gap between the pressure roll and the packages within 1 mm. The actual variance of the gap, however, amounted to 0.3 mm.

After the packages of the first group were doffed, the winder was adjusted so that the spindle had a deviation A of 1/1000 relative to the pressure roll. Packages of a second group were formed in the same manner as before. In this case, the variance of the gap was kept within 0.1 mm throughout the winding operation.

The two groups of the resultant package were evaluated in relation to the hardness and the unwinding tension. The results are listed in Table 3.

From the table, it is apparent that the hardness and the unwinding tension of the packages largely fluctuated in the case of the first group compared to the second group according to the present invention.

## Claims

1. A square-end cheese type yarn package (1) comprising a bobbin (6) and a continuous yarn wound on the bobbin with a plurality of yarn traces imparted by repeated traverses, a traverse being repeated every n cycles, characterized in that with carbon filament yarn (Y) being wound the shifting ratio of the yarn traces lies within a range of from 50% to 150% relative to the average width of the yarn on the package (1) and n is an integer from 1 to 9.

2. A yarn package according to claim 1, in which the shifting ratio is within a range of from 75% to 125% relative to the average yarn width on the package.

3. A yarn package according to claim 1 or claim 2, in which n is between 2 and 6 inclusive.

4. A yarn package according to any one of claims 1 to 3, in which the package has an initial winding angle of not more than 30° and a final winding angle of not less than 4°.

5. A yarn package according to any one of claims 1 to 4, in which the initial winding angle is not less than 10° and the final winding angle is not more than 12°.

6. A yarn package according to claim 5, in which the initial winding angle is not more than 17°.

7. A yarn package according to claim 5 or claim 6, in which the final winding angle is not less than 5°.

8. A yarn package according to any one of claims 1 to 7, in which the average yarn width is within a range of from 1 mm to 5 mm.

9. A yarn package according to claim 8, in which the average yarn width is within a range of from 2 mm to 4 mm.

10. A yarn package according to any one of claims 1 to 9, in which the wound yarn volume of the package (1) is more than 0.04 kg per cm of package width and the hardness of the package within a range of from 50° to 85°, as measured by a Model C Hardness Tester provided by Kobunshi Keiki Seisakusho, Japan.

11. A yarn package according to claim 10, in which the hardness is within a range of from 65° to 75°.

12. A yarn package according to any one of claims 1 to 11, in which the carbon filament yarn (Y) originates from acrylonitrile synethetic fibers.

13. A yarn package according to any one of claims 1 to 12, in which the carbon filament yarn (Y) has a total denier of about 3600 and the shifting ratio is within a range of from 50% to 100%.

14. A yarn package according to any one of claims 1 to 12, in which the carbon filament yarn (Y) has a total denier of about 7200 and the shifting ratio is within a range of from 100% to 150%.

15. A method for forming a square-end cheese type yarn package (1) with a constant winding ratio by utilizing a spindle drive winder comprising a positively rotatable spindle (3) supported in a cantilever manner, a bobbin (6) fitted on the spindle (3), a freely rotatable pressure roll (4) provided along the spindle (3), and a yarn traversing guide (5) for reciprocating the yarn parallel to the axis of the bobbin (6), wherein the winding ratio (i.e. the number of revolutions of the bobbin during one cycle of yarn traverse along the bobbin) is selected so that a yarn trace on the package (1) formed by the traverse is repeated every n cycles, characterized in that for winding carbon filament yarn (Y) the yarn trace formed has a shifting ratio within a range of from 50% to 150% relative to the average yarn width on the package and n is an integer selected from 1 to 9.

16. A method according to claim 15, in which the package (1) is formed under an initial winding tension within a range of from 0.03 grams/D to 0.3 grams/D and a final winding tension within a range of from 0.015 grams/D to 0.3 grams/D, D being the total denier of the yarn to be wound.

17. A method according to claim 16, in which the initial tension is within a range of from 0.07 grams/D to 0.2 grams/D and the final tension is within a range of from 0.03 grams/D to 0.2 grams/D.

18. A method according to any one of claims 15 to 17, in which the spindle (3) has an effective length of more than 400 mm and on which a plurality of bobbins (6) are mounted to form packages (1 each of which has a wound yarn volume of more than 0.04 kg per cm in package width, and a deviation of the spindle (3) relative to the pressure roll (4) is within a range of from 1/5000 to 1/500.

19. A method according to claim 18, in which a gap between the pressure roll and the surfaces of the packages is kept within 2 mm and a variance thereof is kept within 0.2 mm.

## Patentansprüche

1. Garnwickel (1) vom Kreuzspulen-Typ mit quadratischem Ende, der eine Spule (6) und einen fortlaufenden Faden umfaßt, der mit einer Vielzahl von Fadenlinien, die durch wiederholte Hübe übertragen wurden, auf die Spule aufgewickelt ist, wobei jeder Hub aller n Zyklen wiederholt wird, dadurch gekennzeichnet, daß bei einem aufgewickelten Kohlenstoffilament-Faden (Y) das Verschiebungsverhältnis der Fadenlinien, bezogen auf die Durchschnittsbreite des Fadens auf dem Garnwickel (1), im Bereich von 50 bis 150% liegt und n eine ganze Zahl von 1 bis 9 ist.

2. Garnwickel nach Anspruch 1, worin das Verschiebungsverhältnis, bezogen auf die durchschnittliche Fadenbreite auf dem Garnwickei, im Bereich von 75 bis 125% liegt.

3. Garnwickel nach Anspruch 1 oder 2, worin n zwischen 2 und einschließlich 6 liegt.

4. Garnwickel nach einem der Ansprüche 1 bis 3, worin der Garnwickel einen Anfangs-Wicklungswinkel von nicht mehr als 30° und einen End-Wicklungswinkel von nicht weniger 4° aufweist.

5. Garnwickel nach einem der Ansprüche 1 bis 4, worin der Anfangs-Wicklungswinkel nicht kleiner als 10° ist und der End-Wicklungswinkel nicht mehr als 12° beträgt.

6. Garnwickel nach Anspruch 5, worin der Anfangs-Wicklungswinkel nicht mehr als 17° beträgt.

7. Garnwickei nach Anspruch 5 oder 6, worin der End-Wicklungswinkel nicht weniger als 5° beträgt.

8. Garnwickel nach einem der Ansprüche 1 bis 7, worin die durchschnittliche Fadenbreite im Bereich von 1 mm bis 5 mm liegt.

9. Garnwickel nach Anspruch 8, worin die durchschnittliche Fadenbreite im Bereich von 2 mm bis 4 mm liegt.

10. Garnwickel nach einem der Ansprüche 1 bis 9, worin das gewickelte Fadenvolumen auf dem Garnwickel (1) größer als 0,04 kg/cm Garnwickelbreite liegt und die Härte dieses Garnwickels im Bereich von 50° bis 85° liegt, gemessen durch ein Prüfgerät vom Typ "Model C Hardness Tester", geliefert von Kobunshi Keiki Seisakusho, Japan.

11. Garnwickel nach Anspruch 10, worin die Härte im Bereich von 65° bis 75° liegt.

12. Garnwickel nach einem der Ansprüche 1 bis 11, worin der Kohlenstoffilament-Faden (Y) von synthetischen Acrylonitrilfasern abstammt.

13. GarnwiεkeI nach einem der Ansprüche 1 bis 12, worin der Kohlenstoffilament-Faden (Y) ein Gasamt-Denier von etwa 3600 aufweist und das Verschiebungsverhältnis im Bereich von 50% bis 100% liegt.

14. GarnwiεkeI nach einem der Ansprüche 1 bis 12, worin der Kohlenstoffilament-Faden (Y) ein Gesamt-Denier von etwa 7200 aufweist und das Verschiebungsverhältnis im Bereich von 100% bis 150% liegt.

15. Verfahren zur Bildung eines Garnwickels (1) vom Kreuzspulentyp mit quadratischem Ende mit konstantem Wicklungsverhältnis unter Verwendung eines Spindelantriebswicklers, welcher umfaßt: eine positiv drehbare Spindel (3), die freitragend gehalten wird, eine Spule (6), die auf die Spindel (3) angepaßt ist, eine frei drehbare Druckwalze (4), die entlang der Spindel (3) vorgesehen ist, und eine Fadenhubführung (5) zum Hin- und Hergehen des Fadens parallel zur Achse der Spule (6), wobei das Wicklungsverhältnis (und zwar die Anzahl der Umdrehungen der Spule während eines Zyklus des Fadenhubs entlang der Spule) so ausgewählt ist, daß die durch den Hub gebildete Fadenlinie auf dem Garnwickel (1) aller n Zyklen wiederholt wird, dadurch gekennzeichnet; daß zum Wickeln von Kohlenstoffilament-Faden (Y) die gebildete Fadenlinie ein Verschiebungsverhältnis, bezogen auf die durchschnittliche Fadenbreite auf dem Garnwickel, im Bereich von 50% bis 150% aufweist und n eine ganze Zahl von 1 bis 9 ist.

16. Verfahren nach Anspruch 15, worin der Garnwickel (1) bei einer Anfangs-Wicklungsspannung im Bereich von 0,03 g/D bis 0,3 g/D und einer End-Wicklungsspannung im Bereich von 0,015 g/D bis 0,3 g/D gebildet wird, wobei D die Gesamt-Denier des zu wickelnden Fadens darstellt.

17. Verfahren nach Anspruch 16, worin die Anfangsspannung im Bereich von 0,07 g/D bis 0,2 g/D und die Endspannung im Bereich 0,03 g/D bis 0,2 g/D betragen.

18. Verfahren nach einem der Ansprüche 15 bis 17, worin die Spindel (3) eine effektive Länge von größer als 400 mm aufweist und auf ihr eine Vielzahl Spulen (6) zur Ausbildung von Garnwickeln (1) befestigt sind, wobei jede davon ein gewickeltes Garnvolumen von mehr als 0,04 kg pro cm Garnwickelbreite aufweist und die Abweichung der Spindel (3), bezogen auf die Druckwalze (4), im Bereich von 1/5000 bis 1/500 liegt.

19. Verfahren nach Anspruch 18, worin der Spalt zwischen der Druckwalze und den Oberflächen der Garnwickel innerhalb 2 mm gehalten wird und deren Abweichung innerhalb 0,2 mm gehalten wird.

## Revendications

1. Pelote (1) du type croisé à extrémité carrée comprenant une bobine (6) et un filé continu enroulé sur la bobine avec une multitude de tracés de filé conférés par des va-et-vient répétés, un va-et-vient étant répété tous les n-cycles, caractérisée en ce que le filé (Y) en filaments de carbone étant enroulé, le rapport de décalage des tracés de filé est compris entre 50% et 150% par rapport à la largeur moyenne du filé sur la pelote (1), et n est un nombre entier compris entre 1 et 9.

2. Pelote selon la revendication 1, dans laquelle le rapport de décalage est compris entre 75% et 125% par rapport à la largeur moyenne du filé sur la pelote.

3. Pelote selon la revendication 1 ou la revendication 2, dans laquelle n est compris entre 2 et 6 inclus.

4. Pelote selon l'une quelconque des revendications 1 à 3, dans laquelle la pelote a un angle initial d'enroulement non supérieur à 30° et un angle final d'enroulement non inférieur à 4°.

5. Pelote selon l'une quelconque des revendications 1 à 4, dans laquelle l'angle initial d'enroulement n'est pas inférieur à 10° et l'angle final d'enroulement n'est pas supérieur. 12°.

6. Pelote selon la revendication 5, dans laquelle l'angle initial d'enroulement n'est pas supérieur à 17°.

7. Pelote selon la revendication 5 ou la revendication 6, dans laquelle l'angle final d'enroulement n'est pas inférieur à 5°.

8. Pelote selon l'une quelconque des revendications 1 à 7, dans laquelle la largeur moyenne du filé est comprise entre 1 mm et 5 mm.

9. Pelote selon la revendication 8, dans laquelle la largeur moyenne du filé est comprise entre 2 mm et 4 mm.

10. Pelote selon l'une quelconque des revendications 1 à 9, dans laquelle le volume du filé bobiné de la pelote (1) est supérieur à 0,04 kg per cm de largeur de pelote, et la dureté de la pelote est comprise entre 50° et 85°, telle qu'elle est mesurée par un appareil de mesure de dureté du modèle C fourni par la société Kobunshi Keiki Seisakusho, Japon.

11. Pelote selon la revendication 10, dans laquelle la dureté est comprise entre 65° et 75°.

12. Pelote selon l'une quelconque des revendications 1 à 11, dans laquelle le filé (Y) en filaments de carbone a pour origine les fibres synthétiques en acrylonitrile.

13. Pelote selon l'une quelconque des revendications 1 à 12, dans laquelle le filé (Y) en filaments de carbone a un denier total d'environ 3600 et le rapport de décalage est compris entre 50% et 100%.

14. Pelote selon l'une quelconque des revendications 1 à 12, dans laquelle le filé (Y) en filaments de carbone a un denier total d'environ 7200 et le rapport de décalage est compris entre 100% et 150%.

15. Procédé pour former une pelote (1) du type croisé à extrémité carrée avec un rapport d'enroulement constant en utilisant un bobinoir à entraînement par broche comportant une broche (3) pouvant tourner positivement supportée en porte-à-faux, une bobine (6) montée sur la broche (3), un rouleau de compression pouvant tourner librement (4) prévu le long de la broche (3) et un guide (5) pour animer le filé d'un mouvement de va-et-vient parallèlement à l'axe de la bobine (6), dans lequel le rapport d'enroulement (c'est-à-dire le nombre de tours de la bobine pendant un cycle de va-et-vient du filé le long de la bobine) est choisi de façon que le tracé de filé sur la pelote (1) formé par le va-et-vient se répète tous les n cycles, caractérisé en ce que pour l'enroulement du filé (Y) en filaments de carbone le tracé du filé ainsi formé a un rapport de décalage compris entre 50% et 150% par rapport à la largeur moyenne du filé sur la pelote, et n est un nombre entier choisi entre 1 et 9.

16. Procédé selon la revendication 15, dans lequel la pelote (1) est formée sous une tension initiale d'enroulement comprise entre 0,03 gramme/D et 0,3 gramme/D et une tension finale d'enroulement comprise entre 0,015 gramme/D et 0,3 gramme/D, D étant le denier total du filé à enrouler.

17. Procédé selon la revendication 16, dans lequel la tension initiale est comprise entre 0,07 gramme/D et 0,2 gramme/D et la tension finale est comprise entre 0,03 gramme/D et 0,2 gramme/D.

18. Procédé selon l'une quelconque des revendications 15 à 17, dans lequel la broche (3) a une longueur effective supérieure à 400 mm et sur laquelle une multitude de bobines (6) sont montées pour former des pelotes (1), chacune ayant un volume de filé bobiné supérieur à 0,04 kg par cm en largeur de pelote, et l'écart de la broche (3) par rapport au rouleau de compression (4) est compris entre 1/5000 et 1/500.

19. Procédé selon la revendication 18, dans lequel l'intervalle entre le rouleau de compression et les surfaces des pelotes est maintenu à moins de 2 mm et sa variance à moins de 0,2 mm.
